

# United States Patent Office

3,310,492

Patented Mar. 21, 1967

1

3,310,492

## OILS FOR TWO-CYCLE ENGINES CONTAINING BASIC AMINO-CONTAINING DETERGENTS AND ARYL HALIDES

George J. Benoit, Jr., San Anselmo, Calif., assignor to Chevron Research Company, a corporation of Delaware  
No Drawing. Filed Sept. 8, 1964, Ser. No. 395,032  
9 Claims. (Cl. 252—51.5)

This invention concerns lubricating oils useful primarily in two-cycle engines. More particularly, this invention concerns lubricating oils containing aryl halides and amino-containing lubricating oil detergents.

Since the advent of the second World War, the use of the two-cycle engine has proliferated. With the increase in the numbers of motorcycles, motorscooters, chainsaws, lawnmowers, and outboard engines for recreation and commercial boating, the two-cycle engine has secured a place as a prime power source. Despite the popularity and wide distribution of the two-cycle engine, no effort has been made on a broad commercial scale to provide a gasoline tailored to the two-cycle engine's needs. Rather, the efforts of the industry have been directed toward providing an oil which, when combined with gasoline used for automobiles, would be adapted to the requisites of the two-cycle engine.

The presence of the oil admixed with the gasoline increases the tendency for deposits to collect in the exhaust port and piston crown. The presence of the lead compounds which are usually present in gasoline, leads to spark plug fouling, particularly electrode bridging. Additives are therefore included in the oil to minimize the problems of deposits and spark plug fouling. It is essential that the additives do not interfere with each other's respective functions. That is, the various additives in the oil must not react or interact with each other, so as to reduce their effectiveness or deleteriously affect the oil's properties.

Pursuant to this invention, lubricating oil compositions are provided which are stable for long periods of time and minimize formation of deposits and spark plug fouling, which have an amino-containing amide or imide as the lubricating oil detergent, and an aryl halide as the scavenger.

The amount of halohydrocarbon used in the lubricating oil composition will vary with the particular halohydrocarbon used, the desired degree of performance, the particular fuel with which the lubricating composition is to be mixed, and the proportion in which the fuel and lubricating oil composition is mixed. Preferably, the amount of aryl halide used is such that the final fuel/lubricating mixture will contain between about 2 to 5 theories, more preferably between about 2.5 to 4 theories of halide. Generally, the amount of aryl halide in a lubricating oil composition will be between about 0.1 and 5 weight percent, preferably between 0.5 and 3 weight percent.

When the lubricating oil composition is added to a conventional leaded gasoline, it increases the theories of halide available in the gasoline. All conventional leaded gasolines already contain in addition to the alkyl lead compound, some organohalide to act as a scavenger for the lead. Commonly, about 1 to 1.5 theories of halide are present in such gasolines. While this amount of halide scavenger is about sufficient to deal with deposit problems in a 4-stroke internal combustion engine, it is not adequate in a 2-stroke engine, which is run on a mixture of fuel and lubricant. The effect of incorporating the lubricating oil composition to this invention in fuels for 2-stroke engines is to enhance the available theories of halide, thus minimizing the deposit problem, particularly with spark plugs.

2

The term "theory" is used in the industry to mean the quantity of organohalide required in the fuel or fuel/lubricant mixture to convert (theoretically) all the lead present as tetraalkyl lead into a corresponding lead halide.

5 Although tetraethyl lead is the most popular tetraalkyl lead used, the present compositions may be used with any fuel mixture which contains any of the commonly used tetraalkyl lead compounds, e.g., tetramethyl lead, methyltriethyl lead, etc. While the fuel/lubricant mixtures may contain from about 0.1 to 5 cc./gal. of the tetraalkyl lead, the usual amount of tetraalkyl lead will be in the range from about 1 to 3 cc./gal., and more usually about 1.5 cc./gal.

10 The amount of the amine detergent which is used in the base oil will be from about 0.5 weight percent to about 10 weight percent, more usually about 2 to 7 weight percent.

15 The aryl halides used in this invention are those from about 6 to about 16 carbon atoms, preferably 6 to 12 carbon atoms, having from one to two aromatic rings, either fused or nonfused. Each ring may have from about 1 to 3 halogen substituents of atomic number 17 to 35, i.e., chlorine and bromine; preferably, the aromatic molecule will have a total of from 1 to 4 halogens, particularly preferred, 2 halogens. The aromatic ring may be substituted with lower alkyl groups, i.e., alkyl groups of from 1 to 6 carbon atoms.

20 Illustrative compounds within the above description are chlorobenzene, bromobenzene, o-, m-, p-chlorotoluene, o-, m-, p-bromotoluene, 2-chloro-1,3-xylene, 4-chloro-1,3-xylene, 2-bromo-1,3-xylene, 4-bromo-1,3-xylene, 4,6-dichloro-1,3-xylene, 4,6-dibromo-1,3-xylene, 2,5-dibromo-1,4-xylene, 2,5-dichloro-1,4-xylene, 2-bromo-5-chloro-1,4-xylene, 1,2-dibromobenzene, 1,2-dichlorobenzene, 1,4-dibromobenzene, 1,4-dichlorobenzene, 1-bromo-4-chlorobenzene, 2,4-dibromocumene, 4,4'-dibromobiphenyl, etc.

25 Also included in the lubricating oil is the carboxamide or imide of a polyamine. These lubricating oil detergents are reported in a number of domestic and foreign patents, e.g., U.S. Patents Nos. 2,922,708, 3,018,291, 3,024,237, 3,110,673, and French Patent No. 1,265,086. The polyamine will have from 2 to 6 amino groups and a molecular weight in the range from about 60 to about 40 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 94

tions thereof, but are preferably aliphatic. Depending on the structure of the particular acids and amines used in the reaction, amides, imides or imidazolines may be formed.

The preferred monocarboxylic acids will generally be of from 5 to 30 carbon atoms, preferably from 12 to 20 carbon atoms. Such acids are exemplified by caprylic acid, capric acid, lauric acid, myristic acid, palmitic acid, stearic acid, arachidic acid, oleic acid, linoleic acid, abietic acid, etc.

The preferred dicarboxylic acids are the alkenyl succinic acids. Usually, they are used in the reaction as anhydrides, i.e., alkenyl succinic anhydrides, having the following formula:



wherein R is an alkenyl group most conveniently obtained by polymerizing an olefin having from about 2 to 5 carbon atoms. The molecular weight of the resulting polymer would generally be in the range of about 400 to 3000, more usually in the range of about 900 to 1200. Useful olefins are illustrated by ethylene, propylene, 1-butene, 2-butene, isobutene, 1-pentene, and mixtures thereof, preferably isobutene. The methods of polymerizing such olefins to the polymers of the designated molecular weight are well known in the art and do not require exemplification here. As for preparing the alkenyl succinic anhydrides by reaction of the polyolefin and maleic anhydride, this reaction has been repeatedly published in numerous patents, e.g., U.S. Patents Nos. 3,018,250 and 3,024,195.

When referring to carboxylic acids, it is intended to include carboxylic acids and derivatives which will react with amines to form amides, imides or imidazolines. These acyl derivatives include acyl halides, carboxylic acids, anhydrides and esters. The preferred carboxylic acid derivatives are the carboxylic acid itself and the anhydride. However, in particular instances, the other derivatives may find use. The esters which find use are lower alkyl esters, e.g., methyl, ethyl and propyl.

Depending upon the particular carboxyl or acyl derivative used in the reaction with the polyamine, the temperature will range from about 200° F. to about 500° F., more usually from about 275° to 450° F. The pressure used in the system will generally be atmospheric, although in specific instances higher or lower pressures may be used.

The carboxyl equivalents will be at least one fewer than the number of available primary and secondary amino groups. That is, if X is the number of available amino groups, i.e., primary and secondary, then at least one mole and not more than X-1 mole of carboxylic acid—particularly monocarboxylic acid—will be used per mole of polyamines. The equivalent ratio between carboxyl groups and available amino groups will generally be in the range of about .16 to .8 carboxyl equivalent per available amino group.

When the lubricating oil detergent is a polyamide of the alkylene polyamine:



wherein m is an integer of from 1 to 5 and n is an integer of from 1 to 6, the equivalents of carboxylic acid used will be in the range 1 to n.

The amide or polyamide produced from monocarboxylic acid can be characterized by the following formula:



wherein m and n are as defined previously, R<sup>1</sup> is a carboxyl group of from 5 to 30 carbon atoms, and p is an

integer of from at least 1 and not more than n. When n is from 4 to 5, preferably p is from 2 to 3.

The imide from the alkenyl succinic acid with the alkylene polyamine is characterized by the following formula:



where m, n and R are as defined previously. Preferred n varies from 2 to 5, particularly preferred is n equal to 4.

The formation of the amide or imide may be run in the presence or absence of an inert solvent. Inert solvents or dispersants include aromatic hydrocarbons, aliphatic hydrocarbons, specifically mineral oils of lubricating viscosity, aryl halohydrocarbons, ethers and polyethers, etc.

The reaction time will usually be in excess of two hours and rarely exceed 24 hours. More usually, the reaction time will be in the range of about 3 to 15 hours.

The reaction is usually carried out in an inert atmosphere, such as nitrogen, helium, argon, etc., that is in the absence of oxygen. During the reaction it is generally desirable to distill off the water or alcohol (when using an ester) as it is formed. This can be conveniently done by means of a Dean-Stark trap. Desirably, the pressure of the system may be reduced below atmospheric to facilitate the removal of the water.

The amine lubricating oil detergent and aryl halide may be combined with a variety of lubricating oils. Illustrative lubricating oils are petroleum derived oils or mineral oil, such as naphthenic base, paraffin base and mixed base lubricating oils; synthetic oils, e.g., alkylene polymers (such as polymers of butylene, 1-decene, etc.), polyesters, etc.

The following examples are offered by way of illustration and not by way of limitation.

#### Example I

A mixture consisting of about 3.7 parts by weight of tetraethylene pentamine (1 mole) and 0.0002 part by weight of a silicone foam inhibitor was charged into a reaction vessel in a nitrogen atmosphere and heated to 250° F. To this mixture was then added 18.2 parts by weight (3 moles) of a hydrocarbon monocarboxylic acid of a narrow equivalent weight range, having an average equivalent weight of 310. The temperature was then raised to 298°-300° F. for a period in excess of one hour, followed by a further increase to 380° F., maintaining the temperature for a period of about 6 to 7 hours, while reducing the pressure to about 28 mm. Hg in order to facilitate the removal of water. At the end of this time, the reaction mixture is cooled, providing the desired basic amino-containing detergent.

#### Example II

A mixture of 84 g. (0.45 mole) of tetraethylene pentamine and 702 g. (0.45 mole) of a polyisobutylsuccinic anhydride, wherein the polyisobutyl radical was derived from a polyisobutene having a molecular weight of about 1000, was blended with agitation at 125° F. in a nitrogen atmosphere. The temperature was increased to 400° F. over a period of one hour. Then the pressure was reduced to about 2 mm. Hg during a period of 30 minutes. The reaction mixture was allowed to reach room temperature while maintaining the reduced pressure. The reaction product contained about 3.8% nitrogen.

The reaction products from Examples I and II were mixed with aliphatic and aromatic halides, the mixture diluted with a mineral oil and maintained at the specified temperature, the basicity and viscosity being measured

repeatedly. The following Table I indicates the results obtained:

The effect of aging on engine performance was also tested. Oil samples of a solvent refined paraffinic base oil containing 5 weight percent of the detergent of Ex-

TABLE I

| Composition <sup>1</sup><br>(wt. percent) | Ex.<br>No. | Scavenger <sup>2</sup> | Wt. Percent<br>of Comp. | Temp.,<br>°F. | Base No. <sup>3</sup> |         |         |         | Viscosity at 100° F., SSU |         |         |         |
|-------------------------------------------|------------|------------------------|-------------------------|---------------|-----------------------|---------|---------|---------|---------------------------|---------|---------|---------|
|                                           |            |                        |                         |               | 0 Day                 | 20 Days | 30 Days | 40 Days | 0 Day                     | 20 Days | 30 Days | 40 Days |
| Concentrates:                             |            |                        |                         |               |                       |         |         |         |                           |         |         |         |
| 50 I; 50 oil                              | A          |                        |                         | { 70<br>150   | 40<br>40<br>36<br>35  |         | 40      |         |                           |         |         |         |
| 50 I; 39.2 oil                            | B          | p-DBB                  | 10.8                    | { 70<br>150   | 40<br>40<br>38        |         |         | 40      | 700                       |         |         | 700     |
| 50 I; 41.4 oil                            | C          | EDB                    | 8.6                     | { 70<br>150   | 40<br>40              |         |         |         | 700                       |         |         | 700     |
| 50 I; 43.1 oil                            | D          | p-DCB                  | 6.9                     | { 70<br>150   | 40<br>40              |         |         |         | 40                        | 700     |         | 5,000   |
| 47 II; 49 oil                             | E          | p-DBB                  | 3.7                     | { 70<br>150   | 15<br>15              |         |         |         | 700                       |         |         | 700     |
| 47 II; 49 oil                             | F          | EDB                    | 3.0                     | { 70<br>150   | 15<br>15              |         | 7       |         | 15                        |         |         | 700     |
| Finished Oils:                            |            |                        |                         |               |                       |         |         |         |                           |         |         |         |
| 5 I; 95 oil                               | G          | p-DCB                  | 0.68                    | { 70<br>150   | 3.9<br>3.9            |         |         |         | 3.8                       |         |         |         |
| 5 I; 95 oil                               | H          | EDB                    | 0.86                    | { 150         | 4.5                   | 4.6     |         |         | 3.6                       |         |         |         |
| 5 I; 95 oil                               | I          | p-DBB                  | 1.08                    | { 70<br>150   | 3.9<br>3.9            |         |         |         | 3.8                       |         |         |         |
| 5 I; 95 oil                               | J          | 1,2,4-TCB              | 0.55                    | { 70<br>150   | 3.8<br>3.8            |         | 3.7     |         | 3.0                       |         |         |         |
| 5 I; 95 oil                               | K          | o-DCB                  | 0.68                    | { 150         | 3.8<br>3.8            |         | 3.7     |         |                           |         |         |         |

<sup>1</sup> Indicates wt. percent of product from Examples I and II mixed with a Mid-Continent 100 Neutral Oil.

<sup>2</sup> p-DBB = para-dibromobenzene.

p-DCB = para-dichlorobenzene.

o-DCB = ortho-dichlorobenzene.

EDB = ethylenedibromide.

1, 2, 4-TCB = 1, 2, 4-trichlorobenzene.

<sup>3</sup> This base number is essentially that described in method ASTM D-664 except that a larger sample is used, in order to increase the accuracy of the titration.

<sup>4</sup> 16 days.

The aromatic halides were also tested in an engine. The test employs a model 850 Mercury outboard engine, 6-cylinder, 76 cubic inch, 85 H.P., running at 5000 r.p.m. for 100 hours, wide open throttle. An engine is shut down only for spark plug replacement or mechanical trouble. It consists essentially of three 2-cylinder engines in one block equipped with three carburetors, so that three fuel/oil combinations can be run simultaneously.

The engine is mounted in a tank and is equipped with a special test wheel in place of a propeller. Cylinder head temperatures, water in and out temperatures, engine speed and fuel flow rate are recorded.

At the end of the test, inspections are made on the piston rings, piston ring grooves, land, skirt, head and underhead deposits, intake and exhaust port deposits and cylinder head deposits. Ring sticking is reported as F for free (no sticking) or the arc which is stuck (360° being totally stuck). Piston varnish is rated from 0-10, 10 being completely clean. The other deposits are reported on a rating of 50 as being clean and 0 completely covered.

A 2-cycle engine motor oil was prepared by blending California base SAE 40 base oil containing 5 weight percent of the reaction product of Example I, and 0.68 weight percent of p-dichlorobenzene. This amount of p-dichlorobenzene provided one additional theory of halogen for gasoline leaded to 1.5 cc. per gallon of tetraethyl lead and used at a fuel to oil ratio of 20: 1.

The gasoline with which the above-identified motor oil was blended in the fuel to oil ratio 20:1 had an ASTM D-86 distillation starting point of 95° F., a 50 percent point of 219° F. and an end point of 393° F. The gasoline contained 1.5 cc. of tetraethyl lead per gallon of gasoline and one theory of ethylene dibromide scavenger.

The following Table II indicates the results obtained:

ample I and scavenger in the indicated amounts were aged by heating each sample for about 1 month at 170° F.

The test employed a McCulloch chain saw engine, model No. 1-81, run at maximum power for 10 hours, with a head temperature of 440° F. The feed was a 20/1 volume ratio of fuel to oil.

When the run was completed, the piston was removed and inspected for piston varnish, ring sticking (or degree of deposits in groove, if second ring was not stuck), ring land deposits, underhead deposit and exhaust port plugging. A rating of 0-50 is used with 50 as clean.

The following table indicates the results obtained:

TABLE III

|                   | Scavenger | Weight per-<br>cent in Oil <sup>1</sup> | Overall<br>Engine<br>Rating |
|-------------------|-----------|-----------------------------------------|-----------------------------|
| Ethylenedibromide |           | 0.86                                    | <sup>2</sup> 15.6           |
| p-Dichlorobenzene |           | 0.68                                    | 38.5                        |
| p-Dibromobenzene  |           | 1.1                                     | 37.3                        |

<sup>1</sup> Equimolar amounts of the scavenger were used.

<sup>2</sup> The engine was shut down after 6 hours because of excessive deposits.

It is evident that the aryl halides in combination with the polyamine detergents provide excellent results in the two-cycle engines. The engines are kept clean and the rings unstuck under extremely rigorous test conditions. Moreover, both the concentrates and the finished oil composition are stable for long periods of time, retaining their detergent and scavenger ability.

As will be evident to those skilled in the art, various modifications on this process can be made or followed, in the light of the foregoing disclosure and discussion, without departing from the spirit or scope of the disclosure or from the scope of the following claims.

I claim:

1. A 2-cycle engine lubricating oil composition comprising:  
a major proportion of an oil of lubricating viscosity, from about 0.5 to about 10 weight percent of a lubricating oil detergent having at least one free amino group and being the reaction product of a hydrocarbon polyamine of from 2 to 6 amino groups and a

TABLE II

|                    |      |      |
|--------------------|------|------|
| Piston Varnish     | 9.3  | 9.1  |
| Ring Sticking, °F. | 80   | 90   |
| Ratings            | 41.9 | 37.9 |
| Average Rating     | 39.6 |      |

hydrocarbon carboxylic acid of from 1 to 2 carboxyl groups and of from 150 to 1500 equivalent weight, reacted at a temperature in the range of 200° to 500° F.,

and from about 0.1 to 5 weight percent of an aryl halide of from 6 to 10 carbon atoms, wherein the halogen of said halide is of atomic number 17 to 35.

2. A 2-cycle engine lubricating oil composition comprising:

a major proportion of an oil of lubricating viscosity; 10 from about 0.5 to 10 weight percent of a lubricating oil detergent of the following formula:



15

wherein  $m$  is an integer of from 1 to 5,  $n$  is an integer of from 1 to 6,  $p$  is an integer of from 1 to  $n$  and  $R^1$  is a hydrocarbon carboxacyl group of from 5 to 30 carbon atoms; and from 0.1 to 5 weight percent of an aryl halide of from 6 to 10 carbon atoms, wherein the halogen is of atomic number 17 to 35.

3. A composition according to claim 2 wherein  $n$  is 4, and  $p$  is an integer of from 2 to 3.

4. A composition according to claim 3 wherein said aryl halide is dichlorobenzene.

5. A composition according to claim 3 wherein said aryl halide is dibromobenzene.

6. A 2-cycle engine lubricating oil composition comprising:

a major proportion of an oil of lubricating viscosity; from about 0.5 to 10 weight percent of a lubricating oil detergent of the following formula:

25

20

30

35



wherein  $m$  is an integer of from 1 to 5,  $n$  is an integer of from 1 to 6, and  $R$  is an alkenyl group having a molecular weight in the range from about 400 to 3000, and from 0.1 to 5 weight percent of an aryl halide of from 6 to 10 carbon atoms, wherein the halogen is of atomic number 17 to 25.

7. A composition according to claim 6 wherein  $R$  is an alkenyl group of molecular weight in the range from about 900 to 1200.

8. A composition according to claim 7 wherein said aryl halide is dichlorobenzene.

9. A composition according to claim 7 wherein said aryl halide is dibromobenzene.

#### References Cited by the Examiner

##### UNITED STATES PATENTS

|           |         |                 |            |
|-----------|---------|-----------------|------------|
| 3,083,162 | 3/1963  | Lawrence        | 44—58 X    |
| 3,110,673 | 11/1963 | Benoit          | 252—51.5   |
| 3,192,910 | 7/1965  | Coffield et al. | 252—51.5 X |
| 3,216,936 | 11/1965 | Le Suer         | 44—58 X    |
| 3,219,666 | 11/1965 | Norman et al.   | 252—51.5 X |

##### FOREIGN PATENTS

219,994 1/1958 Australia.

DANIEL E. WYMAN, Primary Examiner.

P. P. GARVIN, Assistant Examiner.